

# UNITED STATES PATENT OFFICE.

BENJAMIN F. PYLE, OF DENVER, COLORADO, ASSIGNOR TO THE PYLE METAL-LURGICAL COMPANY, OF DENVER, COLORADO, A CORPORATION OF COLORADO.

## FLUX.

1,416,871.

Specification of Letters Patent. Patented May 23, 1922.

No Drawing.

Application filed December 6, 1919. Serial No. 343,115.

*To all whom it may concern:*

Be it known that I, BENJAMIN F. PYLE, a citizen of the United States, residing at Denver, in the county of Denver and State of Colorado, have invented new and useful Improvements in Fluxes, of which the following is a specification.

This invention relates to improvements in fluxes particularly intended for making metal alloys from crude ores.

The invention has for its object to produce a flux consisting of ingredients, which will, when added to crude ores during smelting, promote fluidity, and remove the objectionable impurities, in the form of slag, as is usual.

Heretofore certain metals, viz: zinc, copper, tin, tungsten, uranium, vanadium and aluminum, could not be brought into metallic form from crude ores, or even treated ores, to make an alloy, and from actual experiments I have found that my improved flux will permit this to be done. It will be understood that when I say "crude ores" I mean ores that have never been treated.

My improved flux consists of the following ingredients: Soda, potash, fluorite, sodium chloride, silica, charcoal, coke, graphite, carbon.

These ingredients will of course be used in the desired proportions, and may be varied at will. My flux is used in precisely the same manner as other fluxes.

What is claimed is:—

1. The herein described flux consisting of soda, potash, fluorite, sodium chloride, silica, charcoal, coke, graphite, and carbon.

2. A flux, having as ingredients soda, potash, fluorite, silica, charcoal, graphite and carbon.

In testimony whereof I have hereunto set my hand in the presence of two subscribing witnesses.

BENJAMIN F. PYLE.

Witnesses:

Mrs. GEO. M. RUSSELL,  
M. HANLON.